

(No Model.)

S. GROSSIORD.  
IMITATION GEM.

No. 400,450.

Patented Apr. 2, 1889.

FIG. 1.



FIG. 3.



FIG. 2.



FIG. 4.



FIG. 5.



FIG. 6.



FIG. 7.



Attest:  
Philip Barnes,  
Geo. T. Smallwood.

Inventor:  
Samuel Grossiord by  
J. Pollock  
his attorney.

# UNITED STATES PATENT OFFICE.

SAMUEL GROSSIORD, OF LES MOUSSIÉRES, NEAR LES BOUCHOUX, ASSIGNOR  
TO RICHARD A. KIPLING, OF PARIS, FRANCE.

## IMITATION GEM.

SPECIFICATION forming part of Letters Patent No. 400,450, dated April 2, 1889.

Application filed July 11, 1888. Serial No. 279,639. (No model.) Patented in France July 2, 1887, No. 184,378.

*To all whom it may concern:*

Be it known that I, SAMUEL GROSSIORD, of Les Moussières, near Les Bouchoux, Jura, France, have invented a certain Improvement 5 in the Manufacture of Imitation Gems, (for which I have obtained a patent in France, dated July 2, 1887, and numbered 184,378,) of which the following specification is a full, clear, and exact description.

10 This invention has reference to the manufacture of artificial or imitation precious stones; and its object is generally to enhance the brilliancy of the imitation gems, and so to approximate more closely the appearance 15 of genuine stones.

According to the present invention, I employ strass, either colorless or of light hue, and on one side thereof, near the edge, I apply a number of pieces of enamel of a color 20 contrasting to that of the strass, and which may be varied according to the effect desired to be produced. The piece of strass, with its spots of enamel, is then subjected to a partial fusion to unite the two. The enamel thus 25 forms a border of varying width around the edge of the strass, leaving the center of the latter uncovered. The enamel may be properly cut, so as to give a suitable outline or design to the exposed part of the strass—such 30 as a star, for example. The effect of the contrast thus obtained and of the refraction of the rays of light by the darker border of enamel gives the appearance of great brilliancy, closely approaching that which characterizes 35 the diamond and other precious stones. This effect may be greatly enhanced by cutting facets on one or both sides of the stone, and still further by covering the bottom thereof with a coating of a light-refracting medium, 40 such as gilding or silvering or black enamel.

The accompanying drawings, which form part of this specification, show the imitation stone in different stages of manufacture.

As shown in Figures 1 and 2, I apply a number of pieces, *a*, of enamel along the edge of one side of a piece of strass, *A*, the pieces of enamel being close together, but preferably not touching. Upon fusing, the pieces of enamel run together, forming a continuous band 45 or border, which, by cutting, may be given any desired configuration, leaving the middle

part of the piece of strass uncovered, as shown in Figs. 3 and 4, this uncovered field taking the form of a star. Of course the enamel may be so cut as to uncover a design of different 55 outline.

The brilliancy of the stone is greatly enhanced by cutting facets thereon, as shown in Figs. 5 and 6. One or both sides of the stone may be faceted. It is also desirable, 60 though not essential, to cover the back of the stone, or at least the middle part thereof, with a coating, *b*, of a light-reflecting substance, as gilding or silvering. (See Fig. 7.) The most brilliant effects are obtained with 65 black enamel on a colorless strass, and imitation gems suitable for mourning jewelry are thus produced. By employing light-blue strass and enamel of darker blue a good imitation of the star-sapphire is produced. 70

Other modifications may be made without departing from the spirit of the invention.

I claim as my invention—

1. The improvement in the manufacture of imitation gems, which consists in fusing upon 75 one surface of a piece of strass a number of pieces of enamel, forming a ring or border within which the surface of the strass is exposed, substantially as described.

2. An imitation gem consisting of a piece 80 of strass surrounded on one face by a border of enamel of darker hue, within which the surface of the lighter glass is exposed, substantially as described.

3. An imitation gem consisting of a piece 85 of strass surrounded with a border of enamel so disposed as to form a design—such as a star—and having facets cut thereon, substantially as described.

4. The faceted imitation gem composed of 90 strass and enamel, the latter being disposed so as to produce a design—such as a star—of the exposed surface of the strass and having a light-reflecting medium on the back thereof, substantially as described. 95

In witness whereof I have hereunto signed my name in the presence of two subscribing witnesses.

SAMUEL GROSSIORD.

Witnesses:

VICTOR MONIOTTE,  
AMAND RITTER.